

1

2,945,814

## LUBRICANT COMPOSITION

Peter William Brett Semmens and James Denis Summers-Smith, Norton-on-Tees, England, assignors to Imperial Chemical Industries Limited, London, England, a corporation of Great Britain

No Drawing. Filed Feb. 27, 1956, Ser. No. 567,744

Claims priority, application Great Britain Mar. 11, 1955

6 Claims. (Cl. 252—49.9)

This invention relates to compositions of matter which are suitable for use as lubricants of surfaces, especially metal surfaces, moving relative to one another.

Under the particular conditions which may occur at low sliding speeds and high loads and which are known as boundary conditions, the hydrodynamic film which is established between sliding metal surfaces by orthodox lubricants is broken down, and the coefficient of friction between the two surfaces rises considerably. This may give rise to excessive local heating and even to complete seizure of the sliding parts.

In order to overcome this deterioration of orthodox lubricants, it has been proposed to use other substances which are effective lubricants under boundary conditions, and which are usually called boundary lubricants. For example, long chain fatty acids and their esters may be used as boundary lubricants, but these compounds are limited in having a comparatively low upper temperature at which they remain effective.

Improved boundary lubricants have been proposed in our co-pending U.S. application Serial No. 530,213, filed August 23, 1955, and now abandoned, which comprise a polyphosphate compound having as the cation a quaternary ammonium group which is attached to at least one radical which contains at least one alkyl group having six or more carbon atoms, and a liquid vehicle in which the polyphosphate is soluble or dispersible such as a hydrocarbon or siloxane oil, or vegetable oil, or an aliphatic ester, or a mixture of these. In the preparation of these polyphosphate derivatives, it is usual to start with a suitable dihydrogen orthophosphate salt such as potassium dihydrogen orthophosphate and to heat it under suitable conditions to provide potassium polyphosphate, which is further treated to produce the quaternary ammonium polyphosphate.

We have now found that improved boundary lubricants are provided by compositions of matter which include quaternary ammonium orthophosphate salts, without the necessity of conversion to polyphosphate.

According to the present invention therefore we provide improved boundary lubricants which comprise an orthophosphate compound of which the cations comprise one or two quaternary ammonium groups in which the nitrogen is attached to at least one radical which contains at least one alkyl group having six or more carbon atoms, and a vehicle which is a lubricant and in which the orthophosphate is soluble or dispersible, such as hydrocarbon, or vegetable oil, or siloxane oil, or an aliphatic ester, or a polyalkylene glycol, or a grease-like solid, or a mixture of these.

Suitable quaternary ammonium groups include cetyl trimethyl ammonium, cetyl pyridinium, didecyl dimethyl ammonium, stearamidomethyl pyridinium, di-octyl dimethyl ammonium, lauryl benzyl dimethyl ammonium, and beta-para-tert-octyl phenoxyethyl benzyl diethyl ammonium. By selecting the vehicle and adjusting the proportions of the orthophosphate compound, mixtures

2

can be obtained having a wide range of viscosity. The orthophosphates themselves are in general grease-like solids, and they may be present in the boundary lubricants in proportions as little as 3% by weight as for example when castor oil is the vehicle with 3% by weight of di(cetyl pyridinium) monohydrogen orthophosphate when a liquid product is desired. On the other hand, if a solid product with a high proportion of orthophosphate is desired, the vehicle may be for example mineral oil mixed with as much as 80% by weight of, for example, di(cetyl trimethyl ammonium) monohydrogen orthophosphate. In addition to mineral oil and castor oil, other suitable vehicles for use in the present invention include for example polymethyl-phenyl siloxanes, polyalkylene glycols, liquid paraffin, substantially completely halogenated hydrocarbons such as those sold under the British Registered Trademark "Florube" 1, and esters of dicarboxylic acids. The vehicle may also be a solid such as petroleum jelly or solid polymethyl-phenyl siloxane.

Boundary lubricants prepared according to the present invention are particularly effective in the lubrication under boundary conditions of such sliding surfaces as are found in bearings, particularly bearings for stainless steel shafts. The table below gives the coefficient of friction between a pair of mild steel and a pair of stainless steel surfaces sliding under boundary conditions, and it will be seen that in most cases the effectiveness of these boundary lubricants is not reduced by increase in temperature, and in some cases the coefficient of friction decreases with increasing temperature. The maximum temperature at which measurements could be taken on the instrument used was 200° C., but considerable evidence exists which suggest that, subject to the thermal stability of the vehicle, these boundary lubricants are equally effective at higher temperatures than 200° C. This is in striking contrast to boundary lubricants based on fatty acids, which are subject to serious temperature limitations.

Quaternary ammonium orthophosphates suitable for use in the present invention may be prepared as follows.

200 mls. of a 10% solution of the appropriate quaternary ammonium halide, preferably the chloride or bromide, preferably at room temperature, are passed through a column of 250 gms. of a suitable exchange resin such as that sold under the British Registered Trademark "Amberlite" IRA 400, which has been previously activated to give the hydroxyl form by contact with aqueous sodium hydroxide solution. A 10% aqueous solution of orthophosphoric acid is added to the resulting quaternary ammonium hydroxide solution conveniently at room temperature and preferably with mixing. If the monohydrogen orthophosphate salt is required, the addition of orthophosphoric acid is stopped when the pH of the solution is 8.5. If however, the dihydrogen salt is required, the addition of orthophosphoric acid is continued until the pH of the solution is 4.5. The solution is then carefully evaporated to dryness, and the product, which is a grease-like solid, is removed.

The quantities and concentrations of quaternary ammonium halide, exchange resin and phosphoric acid are not critical, but the figures given in the above example are convenient values. If the solution of quaternary ammonium halide is too dilute, there will be excessive liquid bulk to handle and evaporate, for a given weight of product. The concentration of the orthophosphoric acid should be sufficiently high to avoid excessive liquid bulk but low enough to give adequate control when the pH of the product solution is adjusted.

In most cases it is necessary to heat the mixture of orthophosphate and vehicle preferably to temperatures below 180° C., and preferably for no longer than 30 minutes. It is also preferable to stir throughout the mixing.

**3**  
**EXAMPLE 1**

0.1 gram of cetyl trimethyl ammonium dihydrogen orthophosphate prepared as hereinbefore described, were mixed with 10 mls. of a mineral oil having a viscosity of 90 centistokes at 20° C. and 4.25 centistokes at 100° C., and heated with constant stirring at 230° C. for 10 min-

5 under boundary conditions using a kinetic boundary friction apparatus, at a relative speed of 0.08 cm. per second, and at 20° to 200° C.

Representative values of the coefficients of friction measured under these conditions are given in the tables below.

**Table 1**

COEFFICIENTS OF FRICTION UNDER BOUNDARY CONDITIONS  
[Sliding speed—0.08 cm./sec.]

| Lubricant         |                 | Austenitic Stainless Steel |        |         |         |         |         |         |         |
|-------------------|-----------------|----------------------------|--------|---------|---------|---------|---------|---------|---------|
|                   |                 | 20° C.                     | 60° C. | 100° C. | 120° C. | 140° C. | 160° C. | 180° C. | 200° C. |
| Vehicle           | Ortho-phosphate |                            |        |         |         |         |         |         |         |
| Nil               | Nil             | 1.11                       | 1.27   | 1.24    | 1.30    | 1.28    | 1.25    | 1.28    | 1.31    |
| 100% M.O.         | Nil             | 0.12                       | 0.16   | 0.16    | 0.29    | 0.32    | 1.12    | 1.16    | 1.20    |
| 99% M.O.          | 1% M.C.A.       | 0.13                       | 0.13   | 0.12    | 0.13    | 0.13    | 0.16    | 0.17    | 0.17    |
| 99% M.O.          | 1% D.C.A.       | 0.12                       | 0.12   | 0.12    | 0.13    | 0.12    | 0.12    | 0.13    | 0.12    |
| 100% Petrol Jelly | Nil             | 0.13                       | 0.17   | 0.18    | 0.18    | 0.20    | 0.20    | 0.21    | 0.29    |
| 93% Petrol Jelly  | 7% M.C.A.       | 0.12                       | 0.11   | 0.10    | 0.09    | 0.09    | 0.07    | 0.06    | 0.05    |
| 93% Petrol Jelly  | 7% D.C.A.       | 0.11                       | 0.10   | 0.10    | 0.08    | 0.07    | 0.06    | 0.05    | 0.06    |

**Table 2**

| Lubricant |                 | Mild Steel |        |         |         |         |         |         |         |
|-----------|-----------------|------------|--------|---------|---------|---------|---------|---------|---------|
|           |                 | 20° C.     | 60° C. | 100° C. | 120° C. | 140° C. | 160° C. | 180° C. | 200° C. |
| Vehicle   | Ortho-phosphate |            |        |         |         |         |         |         |         |
| Nil       | Nil             | 0.82       | 0.92   | 0.88    | 0.83    | 0.94    | 0.92    | 0.87    | 0.95    |
| 100% C.O. | Nil             | 0.09       | 0.10   | 0.12    | 0.12    | 0.14    | 0.14    | 0.14    | 0.15    |
| 95% C.O.  | 5% D.C.P.       | 0.11       | 0.10   | 0.09    | 0.09    | 0.09    | 0.08    | 0.08    | 0.08    |

M.O.—Mineral Oil.  
Viscosity at 20° C., 90 centistokes.

Viscosity at 100° C., 4.25 centistokes.

Density 0.9 gram/c.c. at 10° C.

C.O.—Castor oil.

M.C.A.—Cetyl trimethyl ammonium dihydrogen orthophosphate.

D.C.A.—Di(cetyl trimethyl ammonium) monohydrogen orthophosphate.

D.C.P.—Di (cetyl pyridinium) monohydrogen orthophosphate.

utes. The mixture was then allowed to cool with constant stirring. Most of the orthophosphate dissolved, and the supernatant liquor was decanted from the residue after the mixture was allowed to settle.

**EXAMPLE 2**

An approximately 1% solution of di(cetyl trimethyl ammonium) monohydrogen orthophosphate in mineral oil was prepared by using the same quantities and method just previously described. In this case practically all the orthophosphate dissolved, so that very little residue remained on decanting.

**EXAMPLE 3**

0.7 gram of cetyl trimethyl ammonium dihydrogen orthophosphate prepared according to the method hereinbefore described, and 9.3 grams of petroleum jelly were heated together at 50° C. for 20 minutes with stirring. All the orthophosphate dispersed, and the mixture was allowed to cool.

**EXAMPLE 4**

A dispersion of 0.7 gram of di(cetyl trimethyl ammonium) monohydrogen orthophosphate, prepared according to the method hereinbefore described, in 9.3 grams of petroleum jelly was made in a similar way to the method just previously described.

**EXAMPLE 5**

5 grams of di(cetyl pyridinium) monohydrogen orthophosphate were mixed with 95 grams of castor oil and raised to 140° C. over 5 minutes with constant stirring. The temperature was then raised to 158° C. over 10 minutes, again with constant stirring, and finally the mixture was allowed to cool with stirring. The orthophosphate was completely dissolved in the castor oil.

The compositions just described were tested as lubricants for mild steel and austenitic steel surfaces sliding

We claim:

1. A boundary lubricant selected from the group consisting of lubricant compositions consisting essentially of between about 3 and 80% cetyl trimethyl ammonium dihydrogen orthophosphate dissolved in mineral oil, between about 3 and 80% of di(cetyl trimethyl ammonium) monohydrogen orthophosphate dissolved in mineral oil, between about 3 and 80% cetyl trimethyl ammonium dihydrogen orthophosphate dispersed in petroleum jelly, between about 3 and 80% di(cetyl trimethyl ammonium) monohydrogen orthophosphate dispersed in petroleum jelly, and between about 3 and 80% di(cetyl pyridinium) monohydrogen orthophosphate dissolved in castor oil.

2. A boundary lubricant consisting essentially of between about 3 and 80% of cetyl trimethyl ammonium dihydrogen orthophosphate dissolved in mineral oil.

3. A boundary lubricant consisting essentially of between about 3 and 80% of di(cetyl trimethyl ammonium) monohydrogen orthophosphate dissolved in mineral oil.

4. A boundary lubricant consisting essentially of between about 3 and 80% of cetyl trimethyl ammonium dihydrogen orthophosphate dispersed in petroleum jelly.

5. A boundary lubricant consisting essentially of between about 3 and 80% of di(cetyl trimethyl ammonium) monohydrogen orthophosphate dispersed in petroleum jelly.

6. A boundary lubricant consisting essentially of between about 3 and 80% of di(cetyl pyridinium) monohydrogen orthophosphate dissolved in castor oil.

**References Cited in the file of this patent****UNITED STATES PATENTS**

- 2,285,853 Downing et al. ----- June 9, 1942  
 2,563,506 Werntz ----- Aug. 7, 1951  
 2,592,273 Goebel et al. ----- Apr. 8, 1952  
 2,880,239 Semmens et al. ----- Mar. 31, 1959